

# UNITED STATES PATENT OFFICE.

EDWARD D. GLEASON, OF ASBURY PARK, NEW JERSEY, ASSIGNOR TO NEW-METALS AND PROCESS COMPANY, OF BROOKLYN, NEW YORK, A CORPORATION OF NEW YORK.

## COPPER-LEAD ALLOY.

1,228,017.

Specification of Letters Patent. Patented May 29, 1917.

No Drawing.

Application filed May 17, 1915. Serial No. 28,574.

To all whom it may concern:

Be it known that I, EDWARD D. GLEASON, a citizen of the United States, residing at Asbury Park, in the State of New Jersey, 5 have invented a certain new and useful Improvement in Copper-Lead Alloys, whereof the following is a specification.

Alloys of equal parts of copper and lead may be advantageously employed in bearings 10 because of their plasticity, durability and extremely low coefficient of friction. However, owing to the difference in the melting points and specific gravity of said two metals, such alloys, as ordinarily composed, sweat and 15 segregate in cooling from fusing temperature; so that castings thereof are always more or less irregular in composition and consequently incapable of uniform resistance and wear. Numerous attempts have been made 20 to overcome the difficulties aforesaid, by means dependent upon sudden setting of the alloys and, although such attempts have been more or less successful, such alloys made under the most favorable conditions 25 are only mechanical mixtures wherein the copper in a more or less finely divided state is suspended in a matrix of lead; so that they cannot, under any circumstances, be successfully poured like Babbitt metal or other so 30 called anti-friction metals, because their capacity to set in an abnormally short time does not permit them to flow into small interstices.

Therefore, it is the object of my invention 35 to provide a copper lead alloy which is not a merely mechanical mixture but a homogeneous composition which will set slowly without segregating or sweating and therefore may be used in lieu of Babbitt or other 40 antifriction metal. Moreover, as hereinafter described, my alloy can be made in different degrees of hardness and can, consequently, be employed as a substitute for plastic bronze, having such resistance to shocks and 45 compression as to adapt it for use in bearing boxes for railroad car axles. For instance, my improved alloy containing 60 parts of copper and 40 parts of lead has about the same degree of hardness, by Brinnell test, 50 as a plastic bronze containing 55 parts copper, 5 parts tin, and 40 parts lead, and will withstand the same tensile stress. Moreover, my improved alloy containing 70 parts copper and 30 parts lead is substantially equal 55 in physical characteristics to a bronze con-

taining 65 parts copper, 10 parts tin, and 25 parts lead but has better wearing qualities, when employed as an antifriction bearing, for the reason that the loss of metal by wear, under given conditions, diminishes with the 60 diminution of tin and increase of lead.

An alloy may be conveniently produced in accordance with my invention as follows:—

In a graphite crucible, I fuse 50 parts of 65 copper and, while maintaining it at a temperature above its fusing point, gradually add 50 parts of lead and, when the mixture is liquid throughout its mass, I add a mixture of 3 parts of the native fluorid of sodium and aluminum known as cryolite, and 2 parts manganese oxid. Said oxid is previously reduced by reaction with the fluorin, sodium and aluminum of the cryolite by heating them in the presence of carbon, and 70 the aggregate thereof added to the mixture of copper and lead aforesaid is 5 per cent., by weight. I then cover the entire fused mass in the crucible with a layer of charcoal and when said mass is thoroughly mixed, 75 it may be poured into pigs, for remelting, or directly into sand molds for castings.

The natural fluorid of sodium and aluminum aforesaid varies somewhat in composition; for instance, it may accord with the 85 formula  $Na_3AlF_6$  or the formula  $3NaFAlF_3$ , the latter corresponding to fluorin 54.4, sodium 32.8, and aluminum 12.8 per cent.; or, the formula  $Al_2F_6NaF$ , corresponding to aluminum 13, sodium 32.8, and fluorin 90 54.2 per cent.; or, if what is termed "pure cryolite" it may contain aluminum 13.0, sodium 32.5, and fluorin 54.5, or otherwise, aluminum fluorid 40.25 and sodium fluorid 59.75. 95

Of course, it is unnecessary that the fluorin, sodium and aluminum required for my alloy shall be directly derived from cryolite; and I may reduce the manganese oxid directly, in the presence of carbon, with the 100 molten copper, before adding lead, and, after adding the lead, then add the fluorin, sodium and aluminum.

Of course, in such reduction there is more or less waste, and such loss may be as much 105 as twenty per cent. of the aggregate of the original materials, including such fluorin gas as escapes during the reaction. The involatile portion of such waste matter passes off as a slag.

Therefore, I do not desire to limit myself to the precise details of procedure or to the specific proportions of materials above set forth, as various modifications may be made therein without departing from the essential features of my invention as defined in the appended claims.

I claim:—

- 5 1. The process of making a composition consisting principally of copper and lead; which consists in mixing, at fusing temperature, copper, lead, a manganese derivative, and cryolite.
- 10 2. The process of making a composition consisting principally of copper and lead; which consists in mixing, at fusing temperature, copper, lead, a manganese derivative and fluorid of sodium and aluminum.
- 15 3. The process of making a composition consisting principally of copper and lead; which consists in reducing manganese oxid by fusing the same with cryolite, in the presence of carbon, and adding that composition to a fused mixture of copper and lead.
- 20 4. The process of making a composition consisting principally of copper and lead; which consists in reducing manganese oxid by fusing the same with fluorid of sodium and aluminum, in the presence of carbon, and adding that composition to a fused mixture of copper and lead.
- 25 5. The process of making a composition consisting principally of copper and lead; which consists in fusing copper and, while maintaining it at a temperature above its fusing point, gradually adding an equal

quantity of lead and, when the mixture is liquid throughout its mass, adding a mixture formed by fusing three per cent. of cryolite and two per cent. of manganese 40 oxid.

6. The process of making a composition consisting principally of copper and lead; which consists in fusing copper and, while maintaining it at a temperature above its 45 fusing point, gradually adding an equal quantity of lead and, when the mixture is liquid throughout its mass, adding a mixture formed by fusing three per cent. of fluorid of sodium and aluminum and two 50 per cent. of manganese oxid.

7. The process of making a composition consisting principally of copper and lead; which consists in mixing, at fusing temperature, copper, lead, a manganese derivative, 55 and a fluorin derivative.

8. The process of making a composition consisting principally of copper and lead; which consists in fusing copper and, while maintaining it at fusing temperature, adding 60 lead and, when the mixture is liquid, adding a mixture formed by fusing fluorid of sodium and aluminum and manganese oxid.

In testimony whereof, I have hereunto 65 signed my name at Asbury Park, New Jersey, this sixth day of May, 1915.

EDWARD D. GLEASON.

Witnesses:

J. G. COLEMAN,  
ETHEL MATTSON.